

Patented Mar. 21, 1933

1,902,106

# UNITED STATES PATENT OFFICE

ALFRED M. THOMSEN, OF SAN FRANCISCO, CALIFORNIA

## METHOD OF MANUFACTURING PAPER PULP

No Drawing.

Application filed December 11, 1928. Serial No. 325,398.

The object of my invention is not only to get a stronger fibre than that produced from such trees, grasses, and other substances, as are now utilized in the manufacture of paper pulp, but principally to use such substances as do not produce good pulp by existing processes. Such materials are: Saw-mill wastes of all description, mixtures of woods, sugar-cane bagasse, corn-stalks, barks, and a great 10 series of trees, for example redwood, which do not yield commercial pulp by means now available.

In general, such substances are resolved into fibres by either an acid or an alkali method. In the former, the active substance employed is sulphur dioxide in combination with some base or mixtures of bases; in the latter, the active substance is either caustic soda or a mixture of caustic soda and sodium sulphide. Sodium sulphide as the sole active agent is not employed at present although it is far superior to caustic soda or any admixture of the same. The reason for this anomaly is purely economic. Any process 20 using a sodium salt as a cooking medium must be regenerative, e. g., the soda salt must be reclaimed in such form that it may be used again, otherwise the method becomes too expensive.

30 In the present "Sulphate" and "Kraft" processes, sulphate of soda is used as the source of alkali. In the process of reclamation it is converted into a mixture of carbonate and sulphide, and as the carbonate is inactive in the cooking it is converted into the active caustic soda by causticizing the "green liquor", e. g., a mixture of carbonate, sulphide, and sulphate of sodium in solution, by means of lime. The cooking liquor of both 35 processes, therefore, becomes a mixture of caustic soda and sodium sulphide.

40 In my improved method I use as the active agent only sodium sulphide, and as the carbonate formed during each passage of the alkali through the cooking and reclamation

phases would soon swamp the active reagent in inert material I separate the excess carbonate from the "green liquor" by crystallization and the constant removal of these crystals. My cooking alkali therefore becomes a 50 mixture of carbonate, sulphide, and sulphate, to which I constantly add sulphate to make good all losses, and from which I constantly remove the excess of sodium carbonate produced.

55 My process, therefore, consists of the following steps:

(a) Digesting the material containing fibre with a solution containing as alkali a mixture of carbonate, sulphate, and sulphide of sodium;

(b) Separating the spent solution from the pulp;

(c) Evaporating the solution;

(d) Adding sulphate of sodium;

(e) Incinerating the mixed organic and mineral contents of said solution, the latter remaining as ashes;

(f) Dissolving these ashes, which are a mixture of carbonate, sulphide, and sulphate of sodium, and removing the excess carbonate, thus obtaining again a liquor of the same composition as used in (a).

I claim:

1. In the process of manufacturing paper 75 pulp, the method of liberating the fibre by cooking with a liquor containing sodium sulphide as the sole active agent, and separating the fibre from the spent cooking liquor, evaporating said liquor to a syrupy consistency, incinerating it in a reducing atmosphere, dissolving the ashes in water, separating sodium carbonate formed during incinerating by fractional crystallization, and using the resultant mother liquor for making up 80 fresh cooking liquor.

2. In the process of manufacturing paper 85 pulp, the method of liberating the fibre by cooking with a liquor containing sodium sulphide as the sole active agent, and separat- 90

ing the fibre from the spent cooking liquor, evaporating said liquor to a syrupy consistency, adding sodium sulphate, incinerating it in a reducing atmosphere, dissolving the 5 ashes in water, separating sodium carbonate formed during incinerating by fractional crystallization, and using the resultant mother liquor for making up fresh cooking liquor.

In testimony whereof, I have hereunto set  
10 my signature.

**ALFRED M. THOMSEN.**

**15**

**20**

**25**

**30**

**35**

**40**

**45**

**50**

**55**

**60**

**65**